

June 19, 1973

**C. G. SPROULE, JR., ET AL**  
**INGOT MOLD HOT TOP HEAT INSULATION BOARD AND**  
**METHOD OF PREPARING SAME**  
**Filed Oct. 7, 1970**

3,740,240



FIG. I.



FIG. 2.



FIG. 3.



FIG. 4.

**INVENTORS**

BY Smith, Harding  
Earley & Fallmer

## ATTORNEYS

1

3,740,240

**INGOT MOLD HOT TOP HEAT INSULATION BOARD AND METHOD OF PREPARING SAME**  
Charles G. Sproule, Jr., Tredyffrin Township, and Herbert F. Wagner, Jr., Wayne, Pa., assignors to C. G. Sproule and Associates, Inc., Wynnewood, Pa.

Filed Oct. 7, 1970, Ser. No. 78,827

Int. Cl. B28B 7/36

U.S. Cl. 106—38.25

11 Claims

## ABSTRACT OF THE DISCLOSURE

An ingot mold hot top made of light weight heat insulation board, especially adapted for use in regulating the solidification of a molten mass of metal in a mold, is prepared from a composition comprising perlite, cellulose filler material and binder. At least one surface of the resulting material is treated with silica, or other refractory material.

## BACKGROUND OF THE INVENTION

The present invention relates to ingot mold hot tops made of heat insulation material. More particularly, the present invention relates to heat insulation material adapted for use in connection with ingot casting molds and ingot mold hot tops and to the method of preparing said heat insulation material. Prior art hot tops are disclosed in Daley 3,166,807; Demaison 3,106,756; Davidsson 3,076,239; and Shephard, Jr., et al. 3,006,046.

In the formation of steel or other metal ingots, molten metal is poured into an ingot mold, allowed to solidify, and thereafter removed from processing by rolling, stamping, forging, and the like. As the molten metal becomes solidified in the ingot mold it shrinks. Without a feeder head or reservoir of molten metal, referred to in the industry as a "hot top," to supply the ingot with additional metal during this period, shrinkage or contraction cavities known as "pipe" form in the ingot and render the ingot partially or wholly unsatisfactory.

It is essential that solidification of molten metal in an ingot mold be gradual; with the metal initially solidifying at the bottom of the mold and finally solidifying at the top of the mold. If very slow cooling occurs and a hot top is employed, not only can the formation of "pipe" be avoided in the ingot itself, but impurities are permitted to rise to the portion of the ingot that is normally sheared or cropped. Thus, the prime function of the hot top is to supply a well of molten metal to the solidifying ingot as the metal in that ingot cools and shrinks in volume. To maintain the necessary reservoir of metal molten long enough to supply the cooling ingot, the hot top must be uneconomically oversized, or possess excellent heat insulation characteristics, and/or be supplied with a source of heat.

Typically, hot tops consist of cast metal casings lined with relatively thick heat insulating refractory materials, such as refractory bricks, to protect the casing and reduce heat losses. Although such hot tops are known to produce excellent results, they are beset with problems. Relatively thick heat insulating refractory material is often somewhat irregular in shape, making it difficult to obtain a tight fit of the refractory material within the hot top casing and maintain a tight fit over a wide temperature range, thereby permitting metal which is being cast to flow into cracks along joints of the refractory material, which cannot only result in a substantial waste of metal, but can also result in damage to the hot top casing itself upon contact with molten metal. One of the most common problems of this nature is the difficulty of obtaining a smooth junction between the hot top and the ingot mold. Flaws of this type have caused a large amount of ingot top portions to be scrapped.

2

Utilization of seamless hot top linings formed in situ has only substituted one problem for another. The weight of refractory linings has long been regarded as a distinct drawback and this is particularly true when relatively thick hot top linings are cast in situ. Moreover, removal of a monolithic lining is especially difficult and expensive. In order to be economically practical, it has been necessary in the past to reuse not only the hot top but also the hot top lining. This has meant that the refractory lining has had to be removed from both the metal casing and the ingot without damage to the hot top casing, the ingot or the lining.

In the past, the method of forming insulating hot top sideboards has been by forming a slurry of fibrous material in a tank, pouring the slurry into a mold, and then employing expensive vacuum equipment to remove excessive moisture. The resulting "green" sideboard is then placed in a drying oven where it must be completely dried. This procedure has caused manufacturing costs to be high. Accordingly a desideratum has been a heat insulation material which can be easily formed into suitable board shape and which has the following characteristics: good insulation with small heat capacity, exact thickness, light weight, low manufacturing cost, and versatile utility.

30 This invention relates to low volume sinkheads and to hot-top apparatus for the production of ingots with sinkheads of such character. More particularly, the invention relates to the art of hot-topping which insures the continuous feeding of hot cast metal into the ingots, and is concerned directly with the efficient and continuous feeding of such hot metal by the use of smaller amounts of feed metal made possible by controlling the heat losses in said hot tops.

35 In particular this invention relates to hot tops, sideboards, and linings and covers for sideboards and hot tops. In addition, it relates to an inexpensive method of forming and producing these hot tops, sideboards, and linings and covers, which due to their operating temperature and characteristics, furnish a means for controlling the rate of heat flow from the hot top, sideboards, or linings, so as thus to result in the necessity of a much smaller sinkhead and an increased production of good products from the ingots obtained.

40 It is common practice in the production of killed steel ingots to place a suitable hot top, sideboards, and/or covers on each ingot mold to confine the shrinkage cavity to a sinkhead at the top of the ingot and thus minimize the amount of steel that must be discarded in the rolling mill in order to produce products therefrom that are free from pipe and excessive chemical segregation. The prime function of the hot top system is therefore to supply a well of molten metal to the solidifying ingot as the metal in the ingot freezes and shrinks in volume. The hot top 45 itself has a limited efficiency which is dependent upon a number of factors but it must be remembered that upon the final solidification of the ingot there is still metal in the hot top which cannot be used and must therefore be discarded.

45 In the art today it is well recognized that hot top efficiency can be improved by using refractory linings with normal porosities, such as firebrick or castables, and by using high porosity refractories, such as insulating firebrick, both of which will have a lower insulating factor and have a higher specific heat than the materials used herein.

50 It is therefore a prime feature of this invention to provide a preformed board of suitable high temperature insulating materials which will have lower heat storage and lower heat transfer properties so as thereby to reduce and control heat losses. The invention also contemplates

a method of prefabricating boards for hot top systems which will produce more efficient and smaller hot tops with resultant smaller volume sinkheads and thus result in a greater percentage of the ingot weight being convertible into sound products, with a decrease in the loss of metal in the sinkhead contained in the hot top. The method of prefabricating these boards also makes it possible to vary the thickness and the refractoriness of the boards to further control the flow of heat therethrough.

One object of the invention is to provide a hot top which is very light in weight and very economical to make and use, and one which is so inexpensive that it may be discarded after one use. In addition it may be so designed and prefabricated that it is simple to assemble and place in a hot top as a lining, used as sideboards, or used as a hot top itself. In this connection, it may be stated that the width of the shelf that results from the use of this thin prefabricated board for hot topping ingots is kept to a minimum as the material thickness necessary to control the heat is considerably less than the material thickness of the refractories used in the prior art. The end result is to insure good products from the ingot on rolling, and a narrow shelf at the hot top junction of the ingot is an aid to this desired result.

Another object of the invention is to provide a hot top of which the refractoriness of the prefabricated thin, light weight boards may be controlled. This is advantageous in producing a sinkhead with relatively smooth walls. The combination of a narrow shelf at the junction of the ingot and the sinkhead, and a sinkhead with smooth walls makes it possible to roll sound sinkhead metal into a satisfactory end product, thus realizing a greater amount of end product from a given size ingot and sinkhead. This invention also relates to a method of making refractory only the necessary thickness of the board's outside surfaces so as to keep them as thermally efficient as possible.

In the prior art, the normal weight of firebrick and castables is approximately 125 lb. to 135 lb. per cubic foot while the insulating firebrick runs from 45 lb. to 80 lb. per cubic foot. The normal weight of the insulating boards of this invention is from 10 lb. to 14 lb. per cubic foot and said boards furnish a means for producing lighter easier-to-handle hot tops at a much lower cost and still provide a better heat control than is now possible from the use of firebrick, castables, or insulating firebrick.

Another known method of improving hot top efficiency is through the use of exothermic materials in sideboards, hot tops, and linings and covers for hot tops and sideboards. These exothermic materials are relatively expensive to use, so that their cost may outweigh the value of increased ingot yield. They are also often produced on an individual basis from chemically inconsistent by-products which further increases the cost and difficulty of their preparation as well as causing variations in the results obtained through their use. In addition, since the exothermic sideboards, hot tops, and linings and covers are rather poor insulators, much of the heat from the exothermic reaction is wasted. Therefore, there is a need for a material which is free from the above disadvantages, but which is capable of preventing or minimizing the formation of pipes or other detrimental cavities in the metal ingots.

#### SUMMARY OF THE INVENTION

An object of the present invention is to provide an ingot mold hot top of high temperature heat insulating material.

Another object of the present invention is to provide a rigid, heat insulating hot-top material which has low thermal conductivity at high temperatures.

Still another object of this invention is to provide a preformed heat insulating hot-top board which can effectively and efficiently be used to control the shrinkage cavity in an ingot mold during the solidification of molten metal in said mold.

Yet another object of the present invention is to provide a heat insulation hot-top material which is relatively simple and inexpensive to produce, but which can be formed into a light-weight board which has uniform dimensions.

5 A further object of the present invention is to provide a rigid, heat insulating hot-top material for use in lining molten metal contacting portions of ingot molds and/or hot tops which can be removed easily from such molds and/or hot tops and economically discarded after a single use.

10 A still further object of the present invention is to provide a heat insulation material which can efficiently be used as a hot top without the necessity of employing a metal hot top casing.

15 Another object of the present invention is to provide a rigid, high temperature heat insulating material with a heat-destructible binder and an optimum of refractoriness.

20 Another object of the present invention is to provide a rigid, heat insulating material with a heat-destructible binder, an optimum of refractoriness and having low thermal conductivity at high temperatures.

Another object is to provide a preformed heat insulating 25 material with a heat-destructible binder, an optimum of refractoriness having low thermal conductivity at high temperatures and adapted to be placed in or on ingot molds to control the solidification of molten metal therein, thereby preventing or minimizing the formation of pipe 30 or other detrimental cavities in the metal ingots.

Another object is to provide an ingot liner board with a heat-destructible binder and an optimum of refractoriness which is relatively simple and inexpensive to produce, but which is highly effective in use.

35 Another object is to provide a rigid, heat-insulating material with a heat-destructible binder and optimum refractoriness for use in lining molten-contacting portions of ingot molds and/or hot tops.

40 A still further object of this invention is to provide a preformed heat-insulating board with a heat-destructible binder and an optimum refractoriness for metal ingot molds which is relatively inexpensive, both as to the cost of the components of the board and as to the cost of its manufacture, the board providing good heat insulation 45 for the molten metal within the ingot mold.

In accordance with the present invention a heat insulation material is prepared which finds particular application in connection with ingot casting molds and ingot mold hot tops. The composition of such material comprises perlite, cellulose fillers and a binder. The surface of heat insulating board prepared from this material is treated with silica by impregnation or other suitable means. In particular, heat insulating board of the present invention comprises from about 60 to about 80 percent by weight of perlite, from about 5 to about 10 percent by weight of a heat destructive binder, from about 15 to about 30 percent by weight of cellulose filler material. This board is subsequently treated on at least one surface with about 2 to about 50 percent by weight of silica.

#### BRIEF DESCRIPTION OF THE DRAWINGS

Other and further objects, advantages, and features of the invention will be apparent to those skilled in the art from the following detailed description thereof, taken in conjunction with the accompanying drawings, in which:

65 FIG. 1 is a sectional view of the upper portion of an ingot mold provided with a hot top, the metal receiving cavity of the hot top being lined with the novel heat insulating material of the present invention;

70 FIG. 2 is a sectional view of an ingot mold in which the novel heat insulating material of the present invention serves as a hot top for a reservoir of molten metal which feeds the pipe or shrinkage cavity as it tends to 75 form in the solidifying ingot;

FIG. 3 is a sectional view of the top portion of an ingot mold having the novel heat insulating boards of this invention lining the upper portion of the mold cavity; and

FIG. 4 is a sectional view of the top portion of an ingot mold having a lining composed of multiple heat insulating boards of the present invention. In addition, FIG. 4 illustrates the use of the novel heat insulating boards of this invention as a cover for ingot molds during solidification of molten metal within the mold.

#### DESCRIPTION OF THE PREFERRED EMBODIMENTS

According to the present invention, heat insulating material is produced which is especially well adapted to be formed into boards for use in controlling the solidification of molten metal. The composition of the heat insulating material comprises perlite, cellulose fillers and binder and may contain other ingredients, such as clay. These materials are present in the following amounts: from about 60 to about 80 percent by weight of perlite, from about 15 to about 30 percent by weight of cellulose filler material, from about 5 to about 10 percent by weight of a heat destructible binder, such as asphalt binder, and from about 3 to about 6 percent by weight of clay, such as kaolin clay. A typical analysis of the inorganic material present in the composition is shown by the following table:

|                       | Percent by weight |         |
|-----------------------|-------------------|---------|
|                       | Minimum           | Maximum |
| Ferric oxide.....     | 0.05              | 1.5     |
| Titanium dioxide..... | 0.03              | 0.2     |
| Magnesium oxide.....  | 0.1               | 0.5     |
| Silicon dioxide.....  | 71.0              | 75.0    |
| Aluminum oxide.....   | 12.5              | 18.0    |
| Potassium oxide.....  | 4.0               | 5.0     |
| Sodium oxide.....     | 2.9               | 4.0     |
| Calcium oxide.....    | 0.5               | 2.0     |

As previously indicated, at least one surface of the resulting heat insulating material is treated with silica in an amount between about 2 percent by weight and 50 percent by weight, and preferably between about 5 percent by weight and 12 percent by weight.

The dried heat insulating board, i.e. board which is not "green" is impregnated with silica to a depth up to  $\frac{1}{4}$  inch employing any suitable procedure. For example, according to one procedure the board can be dipped into a silica solution and the depth of surface treatment regulated by the depth of the solution, concentration of silica in the solution, and the like. In accordance with another procedure, the board can be sprayed with a silica solution. The silica solution can be simply a dispersion of silica in liquid medium, such as water, such as Du Pont's Ludox, a colloidal silica, submicroscopic particles of silica in colloidal suspension in water, or such as Monsanto's Psyton. If desired, conventional wetting agents such as Du Pont's Alkanol WZN, can be added to the silica solution for further control of the surface treatment. By thus regulating the location of the surface treatment and the depth of impregnation the thermal efficiency of the board can be modified for varying applications. As the amount of silica impregnation is increased, the thermal efficiency of the board decreases. It has also been found that there is a definite relationship between the mass of the sinkhead and the depth of refractory surface treatment necessary to maintain the integrity of the heat insulating board. For example, it has been found that boards of the present invention perform properly when used with a sinkhead of about 200 pounds if they have a surface treatment of about  $\frac{1}{32}$  inch in depth. On the other hand, it has been found that the same boards need a surface treatment of about  $\frac{1}{8}$  inch in depth if used with a sinkhead weighing about 4,000 pounds. After

the board has been treated with silica it is then dried at room temperature or slightly elevated temperatures in an oven prior to utilization.

Heat insulating material having the composition described above provides excellent characteristics when used to control the rate of solidification of a mass of molten metal in an ingot. Due to the low thermal conductivity of this material, the heat of the melt is not dissipated rapidly through the walls of the mold and/or hot top, but is retained in the molten metal. In this manner, there is provided a reservoir of molten metal in the upper portion of a mold or hot top which feeds the pipe or shrinkage cavity as it tends to form in the solidifying ingot, thereby preventing or at least minimizing the formation of pipe in the metal ingot. The heat insulating material of the above composition is substantially incombustible at the temperatures encountered in the production of steel ingots.

The heat insulating board of the present invention not only results in increased ingot yield and improved quality, but results in significant savings in time and labor. Hot tops can be constructed from the heat insulating board which weigh about  $\frac{1}{4}$  to  $\frac{1}{6}$  of the weight of hot tops previously used. Because of their light weight and durability, hot tops formed from the heat insulating board can be easily handled by one man without material handling equipment.

Another advantage of the heat insulating material of the present invention is the fact that boards of the material can be formed relatively inexpensively by conventional procedures, such as the commercial Fourdrinier papermaking machine. Since the heat insulating board is so inexpensive to make, it can be discarded after only one use.

Boards thus formed can be varied in thickness, but are normally prepared in a thickness ranging from  $\frac{1}{2}$  to  $1\frac{1}{2}$  inches. Even though it is possible to prepare such boards in varying uniform thicknesses, it is often advantageous to laminate a number of boards together when thicker boards of heat insulating material are desired. Due to the composition of the heat insulating material, the light weight boards formed from such material are easily trimmed to any desired shape, even when the boards have been laminated together. The strength of the resulting boards is such that they are not susceptible to breakage in handling and they will not change in shape or otherwise deteriorate in storage.

One very useful application for the heat insulating material of the present invention is in the use of such material in hot tops. Referring particularly to FIG. 1, numeral 10 designates an ingot mold which is illustrated in phantom outline. A hot top casing 11, which is normally composed of cast iron, is centered between flanges 12 and 13 which extend from and overlap the upper edge of ingot mold 10. The square hot top casing 11 is lined on all four sides with sidewalls 14 of heat insulating board having a layer 14a of silica. Casing 11 and sidewalls 14 are seated on refractory ring 15 also made of heat insulating board with a layer 15a of silica, so that casing 11 is completely protected from the molten steel being poured into ingot mold 10. A metal "wiper strip" or "chill" 15b may be provided for refractory ring 15, if desired. The hot top casing 11 is also provided with trunnions 16 and 17 which can be used in removing the casing from ingot mold 10 after ingot 18 has solidified. The resulting shrinkage cavity is shown at 19.

Since the heat insulating board of the present invention is structurally quite rigid and can be joined together by a variety of suitable means, such as nailing, it is possible to use the heat insulating board itself without a hot top casing for the purpose of controlling the solidification of molten metal in an ingot. As shown in FIG. 2, a hot top 20 composed solely of heat insulating board with a layer 20a of silica is seated in flange 21 of ingot mold 22, which is illustrated in phantom outline. When

the molten metal in the mold solidifies and ingot 23 is formed, shrinkage cavity 24 occurs in the hot top.

The heat insulating board of the present invention can also be employed in the ingot mold itself when "pipe" in the upper portion of the ingot mold is not objectionable. As shown in FIGS. 3 and 4, the heat insulating board of the present invention can be used to line the upper portion of an ingot in order to reduce the amount of heat radiated from that portion and thereby maintain a reservoir of molten metal until the remainder of the ingot has been completely solidified. The size, shape and location of the shrinkage cavity or "pipe" can thereby be regulated.

Referring specifically to FIG. 3, high temperature board 30 with a layer 30a of silica is shown lining the upper portion of ingot mold 31. Due to the high temperature heat insulating property of board 30, a molten metal reservoir 32 is provided as ingot 33 solidifies in mold 31.

A similar embodiment showing the application of the high temperature board is illustrated by FIG. 4, where two layers of high temperature board 40 and 41 are bonded together and line the upper portion of ingot mold 42. A silica layer 40a is provided to protect bonded boards 40, 41 from contact with the molten metal 45. A third high temperature board 43, having a bottom layer 43a of silica, is employed as a cover while molten metal 44 is solidifying to form ingot 45.

While the invention has been described in terms of the production of heat insulating hot-top board, it will be understood that if desired the heat insulating material of the present invention can be formed into a one piece hot top. The light weight of the heat insulating material permits a unitary hot top to be easily handled by one man and avoids the necessity of joining heat insulating boards together with a U-shaped clip, nails, bolts, a friction fit or any other suitable means. In contrast, a conventional hot top for as small an ingot mold as 22 inches by 22 inches by 80 inches often weighs as much as 120 pounds and cannot be handled by one man without the help of equipment.

By varying the thickness of the insulating board the flow of heat therethrough can be controlled and it is possible to produce more efficient and smaller hot tops with a resultant smaller volume sinkhead and permit a greater percentage of the ingot weight to be converted into sound products. Although the heat insulating board of the present invention is rigid even at thicknesses of less than  $\frac{1}{2}$  inch, it will be understood that the thickness of the heat insulating board decreases it is possible to attach wire mesh or some other suitable material to the heat insulating board to insure that the board will remain in a predetermined form under the conditions in which it is used. For certain applications it is desirable to apply a layer of some other material, such as aluminum, to one side of the heat insulation board or in between heat insulation boards laminated together. It will also be understood that it is not essential for the surfaces of the heat insulating board to be flat and the board may be provided with one or more corrugated surfaces.

If desired, other materials can be included with the heat insulation material. For example, fibrous materials, such as asbestos; mineral wool; alumina powder; and the like can be incorporated.

While it is convenient to form boards of the heat insulating material on a Fourdrinier machine, it is to be understood that such boards can be formed in other ways. For example, heat insulating boards can also be formed by casting a slurry of the heat insulating material in a mold of suitable shape and size. This alternative method of production is not preferred since production costs tend to be higher than when the boards are formed on a Fourdrinier machine. Regardless of the method of production employed, the resulting board of heat insulating material must be treated with finely divided silica in the

percentages indicated above. This impregnation of the board with silica can be done in any convenient manner such as spraying, dipping, and the like using a silica solution. It is not essential that the board be impregnated on both sides with silica since effective maintenance of the high temperature integrity of the product has been observed when the board is impregnated with silica on only one side. This fact is consistent with the observation that greater heat integrity is obtained when the high temperature material is impregnated with silica after formation of the heat insulating material into a board than by the mere incorporation of silica with the other ingredients in the composition used to prepare the high temperature heat insulation board.

The heat-insulating boards of the present invention are relatively inexpensive to use for they are inexpensive both as to the materials employed and the cost of manufacture. Thus, boards of the composition set forth above, due to the types and amounts of materials used, can be made rigid, heat-insulating, with a heat-destructible binder and be made in large sheets in a continuous commercial operation on a conventional Fourdrinier type papermaking machine, and the large sheets cut into boards of any desired shape and size to later be made as refractory as desired. Therefore, it is not necessary to press or cast the boards individually, as with the boards used heretofore, for the heat-insulating boards of the present invention may be made in large quantities in a continuous commercial operation. Generally, in the production of these boards on a Fourdrinier, the individual components are formed into slurries, the slurries transferred to one or more stock chests and pumped to a machine chest from where the stock is flowed onto a moving wire of the machine. Water is subsequently removed from the material on the wire to form a self-supporting sheet which is then pressed, cut into predetermined lengths, and dried to form rigid sheets. The rigid sheets are then trimmed to form heat-insulating boards of a desired shape and size.

The boards thus formed usually have a thickness of from about  $\frac{1}{2}$  to  $1\frac{1}{2}$  inches, plus or minus  $\frac{1}{16}$  inch. Generally, boards of 1 inch thickness are preferred for lining the upper portion of the mold cavity of ingot molds. For some applications, a number of the boards may be laminated together to form thicker boards, bodies or blocks of heat-insulating materials. At this point the boards have a density of from about 9 lb. to 13 lb. per cubic foot, with densities in the range of 10 lb. to 12 lb. per cubic foot being preferred.

From the foregoing it will be seen that this invention is well adapted to obtain all of the ends and objects hereinabove set forth, together with other advantages which are obvious and which are inherent to the system.

It will be understood that various modifications can be made without departing from the invention. Obvious modifications will occur to those skilled in the art and it will therefore be recognized that the invention is not limited to the precise embodiments shown and described.

What is claimed is:

1. In a heat insulating hot-top board comprising perlite, cellulose filler, and a binder of an asphalt type, the improvement comprising having at least one surface of the board coated with about 2 to about 50% by weight of silica.
2. The heat insulating board of claim 1, in which clay is present with the perlite, cellulose fillers and binder.
3. The heat insulating board of claim 1, in which the binder is a heat destructible binder.
4. The heat insulating board of claim 3, in which the heat destructible binder is an asphalt binder.
5. In a method of preparing a heat insulating hot-top board composed of perlite, cellulose filler, and binder, the improvement comprising treating at least one surface of said heat insulating board with from about 2 to about

50% by weight of silica, and then drying the silica treated board.

6. The method of claim 5, in which the heat insulating board is treated with silica by impregnating the board with a silica solution.

7. The method of claim 5, in which the heat insulating board is treated with silica by spraying the board with a silica solution.

8. In a heat insulating hot-top board comprising from about 60 to about 80 percent by weight of perlite, from about 5 to about 10 percent by weight of asphalt binder and from about 15 to about 30 percent by weight of cellulose fillers, the improvement comprising having at least one surface of said board impregnated with from about 2 to about 50 percent by weight of silica.

9. The heat insulating board of claim 8, in which the board is impregnated with silica to a depth of up to  $\frac{1}{4}$  inch.

10. The heat insulating board of claim 8, in which the silica is concentrated on only one surface of the board.

11. In an ingot mold hot-top of lightweight heat insulation article, comprising a plurality of heat insulating hot-top boards arranged in contiguous relationship and adapted to be mounted inside an ingot mold and cover

interior surfaces thereof to protect said interior surfaces from contact by molten metal and to heat insulate said molten metal, said hot-top boards including perlite, cellulose filler and binder, the improvement comprising having at least one surface of the boards coated with about 2 to about 50% by weight of silica.

#### References Cited

##### UNITED STATES PATENTS

|    |           |         |        |       |             |
|----|-----------|---------|--------|-------|-------------|
| 10 | 3,095,347 | 6/1963  | Becker | ----- | 106—122     |
|    | 2,361,386 | 10/1944 | Earys  | ----- | 106—38.8    |
|    | 3,262,165 | 7/1966  | Ingham | ----- | 106—38.22 X |
|    | 3,460,606 | 8/1969  | Boddey | ----- | 106—38.5 R  |

##### FOREIGN PATENTS

|           |        |               |       |           |
|-----------|--------|---------------|-------|-----------|
| 921,976   | 3/1963 | Great Britain | ----- | 249—201   |
| 1,813,772 | 7/1969 | Germany       | ----- | 106—38.22 |

LORENZO B. HAYES, Primary Examiner

U.S. Cl. X.R.

106—38.8, 282; 249—197; 252—62